

No. 836,177.

PATENTED NOV. 20, 1906.

E. D. CHAPLIN.

ART OF PRODUCING PIGMENTS BY ELECTROLYSIS.

APPLICATION FILED FEB. 3, 1906.



WITNESSES =

E. B. Tomlinson.

Patrick J. Conroy.

INVENTOR =

Edwin D. Chaplin

by

Browne & Woodworth

his attorneys.

# UNITED STATES PATENT OFFICE.

EDWIN D. CHAPLIN, OF BOSTON, MASSACHUSETTS.

## ART OF PRODUCING PIGMENTS BY ELECTROLYSIS.

No. 836,177.

Specification of Letters Patent.

Patented Nov. 20, 1906.

Application filed February 3, 1906. Serial No. 299,236.

*To all whom it may concern:*

Be it known that I, EDWIN D. CHAPLIN, a citizen of the United States, and a resident of Boston, in the county of Suffolk and State of Massachusetts, have invented a new and useful Improvement in the Art of Producing Pigments by Electrolysis, of which the following is a specification.

My invention relates to the art of producing pigments by electrolysis; and it relates more particularly to a process for so producing white lead or lead carbonate.

In the manufacture of lead carbonate by electrolysis I prefer to employ an electrolyte which under the influence of the electric current will separate into a solvent of lead and an alkaline hydrate and thereby to produce in the anode-compartment containing metallic lead, which may be the anode of an electrolyzer, a solution of a soluble salt of lead and in the cathode-compartment an alkaline hydrate. I have found it essential to the commercial production of white lead to maintain the lead solution and the alkaline hydrate separate and not to produce any lead precipitate in the electrolyzer itself. I have also found it essential to employ some means, such as an oxidizing agent, to prevent the formation of insoluble salts of lead in the electrolyzer.

A direct process involving the principles above briefly set forth is described in United States Letters Patent No. 675,555, June 4, 1901, granted to H. G. Halloran and myself, and according to said process an oxidizing agent in the form of a soluble chlorate salt is electrolytically formed from a soluble chlorid salt which is mixed with the original electrolyte, a soluble salt of lead is produced in the presence of the said oxidizing agent, and said soluble salt of lead is carbonated directly in any suitable manner.

The object of the present invention is to provide an indirect process of electrolytically producing white lead or one in which the soluble salt of lead is first precipitated to form lead hydrate and said lead hydrate then carbonated to produce white lead. While such indirect process is not so economical as the direct process, I have found that the resulting product differs in molecular structure from that produced by the direct process and that it greatly excels the

latter in color carrying and covering capacity.

55

My invention may best be understood by having reference to the drawing, which accompanies and forms a part of this specification, and which illustrates in diagrammatic form one arrangement of apparatus and circuits whereby my process may be carried into effect; but it is to be understood that my process is broader than mere apparatus and may be carried into effect by a great variety of apparatus and circuit arrangements. 60

65

In the drawing the figure represents an apparatus and system of circuits for electrolytically producing white lead.

70

In the figure, 1 represents the supply-tank containing an electrolyte, which under the influence of the electric current will be separated into a solvent of lead and an alkaline hydrate—such, for example, as an aqueous solution of an alkaline base and containing also an aqueous solution of a chlorid or a chloride of an alkaline base.

75

I shall hereinafter refer to the solution in tank 1 as the "neutral" solution and shall assume that it consists of sodium nitrate and sodium chlorid.

80

3 represents an electrolyzer divided into an anode-compartment 3' and a cathode-compartment 3" by means of the foraminous diaphragms 4 4', between which is formed a compartment for receiving the electrolyte from tank 1 through the pipe 2, which is provided with a valve 2'. For the purpose of preventing a mixture of the anolyte and catholyte in the electrolyzer, and consequently a precipitation of lead hydrate in the electrolyzer, I may maintain a preponderance of pressure on the inner sides of said diaphragms, preferably by maintaining the level of the electrolyte between the diaphragms higher than the level of the anolyte and catholyte. The level of the electrolyte in the compartment between the diaphragms is indicated by the dotted line 9, and the level of the anolyte and catholyte, which is governed by the height of the bends of the outlet-pipes 7 and 8, is indicated by the dotted lines 10 10.

85

In order to prevent said outlet-pipes from siphoning the liquids out of the electrolyzer, the upper portion of each of said bends may be provided with an opening 26 26' to 105 equalize the atmospheric pressure on the col-

100

105

umns of liquid in the two portions of each of said pipes.

The lead to be operated upon is placed in the anode-compartment and may form the 5 anode of the electrolyzer. In the present case the lead is shown in the form of a lead pig 5, connected by the conductor *d* to the positive pole of the dynamo *D* or other suitable source of current. The cathode of the 10 electrolyzer 6 may consist of copper or any other suitable metal and is connected by the conductor *c* to the negative pole of the dynamo.

When the electrolyzer is charged with the 15 neutral solution and the electric current passed therethrough, a soluble acid salt of lead is formed in the anode-compartment 3' and an alkaline hydrate—in the present case assumed above sodium hydrate—is formed in 20 the cathode-compartment 3''. Presumably lead hydrate is at first formed in the anode-compartment, is converted into a lead chlorid, which is soluble at the temperature at which the electrolyte is maintained by the steam-coil 30 or by any other suitable means, and 25 finally is converted into lead oxychlorid, which is soluble at ordinary temperatures. The lead oxychlorid being an acid salt of lead renders impossible the formation of insoluble 30 basic salts of lead. The solution of said acid salt of lead may be discharged into the settling-tank 29 by the pipe 8 and thence into the precipitating-tank 22 by the pipe 21, which is provided with the valve 21', or, as is 35 obvious, it may be discharged directly into said precipitating-tank.

The alkaline hydrate produced in the cathode-compartment 3'' may be discharged into the settling-tank 27 by the pipe 7 and thence 40 into the precipitating-tank 22 by the pipe 20, which is provided with the valve 20', or, as is obvious, it may be discharged directly into said precipitating-tank.

In the tank 22 lead hydrate is precipitated 45 from the acid salt of lead and settles on the filter 23 at the bottom of said tank, while the filtrate, which in the present assumed case consists, probably, of a mixture of sodium nitrate, sodium chlorate, and sodium chlorid, 50 is pumped back to the supply-tank 1 through the pipe 25, provided with the valve 25', by the pump 26.

A portion of the alkaline hydrate formed in the cathode-compartment 3'' is conveyed 55 to the tank 11, either directly from the electrolyzer or from the settling-tank 27 by the pipe 28, provided with the valve 28', and is converted into a bicarbonate of an alkaline base—sodium bicarbonate in the present assumed case—by treating the same with carbon dioxid produced in the generator 12, which connects with the tank 11 by the pipe 13, provided with the valve 13'.

The lead hydrate formed in the tank 22 is discharged by the pipe 24, provided with the 65 valve 24', into the precipitating-tank 15, and the bicarbonate formed in the tank 11 is conveyed into said tank through the pipe 14, provided with the valve 14', thereby converting the lead hydrate into lead carbonate. The 70 lead carbonate so formed settles at the bottom of the tank 15 on the filter 16 and may be drawn off through the pipe 18, run through a filter-press, and prepared for use. The filtrate may be drawn off by the pipe 17.

By means of the indirect process herein described I am enabled to produce white lead of a color carrying and covering capacity which is greatly superior to that produced by the direct process in which the soluble acid salt of 80 lead is directly carbonated. The process is continuous and, in addition to the lead and carbon dioxid consumed, requires only the addition from time to time of fresh quantities of neutral solution.

I claim—

1. As an improvement in the art of producing white lead by electrolysis, the process herein described which consists in electrolytically producing a soluble acid salt of lead, 90 withdrawing the same and precipitating lead hydrate therefrom, and then carbonating said lead hydrate to produce white lead.

2. As an improvement in the art of producing white lead by electrolysis, the process 95 herein described which consists in electrolytically producing a solution of oxychlorid of lead, withdrawing the same and precipitating lead hydrate therefrom, and then carbonating said lead hydrate to produce white lead.

3. As an improvement in the art of producing white lead by electrolysis, the process herein described which consists in electrolytically producing an alkaline hydrate and 105 a soluble acid salt of lead, withdrawing and mixing said alkaline hydrate and said acid salt of lead to precipitate lead hydrate, and then carbonating said lead hydrate to produce white lead.

4. As an improvement in the art of producing white lead by electrolysis, the process herein described which consists in electrolytically producing an alkaline hydrate and a solution of oxychlorid of lead, withdrawing 115 and mixing said alkaline hydrate and oxychlorid of lead to precipitate lead hydrate, and then carbonating said lead hydrate to produce white lead.

5. As an improvement in the art of producing white lead by electrolysis, the process herein described which consists in electrolytically producing an alkaline hydrate and a solution of oxychlorid of lead, withdrawing 120 said oxychlorid of lead, withdrawing and mixing a portion of said alkaline hydrate

with said oxychlorid of lead, thereby precipitating lead hydrate, withdrawing and carbonating another portion of said alkaline hydrate, and then carbonating said lead hydrate with the resulting bicarbonate to produce white lead.

5 In testimony whereof I have hereunto sub-

scribed my name this 5th day of January, 1906.

EDWIN D. CHAPLIN.

Witnesses:

CHARLES C. KURTZ,  
GEO. K. WOODWORTH.